

May 28, 1968

K. W. J. NEALE ET AL

3,385,748

WATER RELEASE TRANSFER

Filed July 15, 1963



1

3,385,748

### WATER RELEASE TRANSFER

Kenneth William James Neale and David Wellings Poin-  
ton, Stoke-on-Trent, England, assignors to Johnson,  
Matthey & Company Limited, London, England, a Brit-  
ish company

Filed July 15, 1963, Ser. No. 295,054  
Claims priority, application Great Britain, July 17, 1962,  
27,390/62

1 Claim. (Cl. 161—6)

This invention relates generally to improvements in and relating to the decoration of heat-resisting bases, that is to say, bases capable of withstanding firing at a temperature of at least 400° C. such as glass, fused silica, or pottery, and is more particularly concerned with the decoration of such bases with a design or decoration in gold by means of decalcomanias or transfers.

A decalcomania or transfer for use in the decoration of a heat-resisting base usually comprises a sheet or backing or absorbent paper carrying a layer of water-soluble gum to which is directly applied either a cellulose support film, which itself carries a design to be applied to the base, or the design itself, which is then covered by a support film, which thus constitutes a covercoat as well as a support for the design after its release from the paper backing and before firing of the base decorated therewith. The design, which may be applied to the transfer paper in any suitable manner, such as by the silk-screen printing method, may consist of a ceramic color or vitrifiable enamel or of a metallic "Lustre" composition, such, for example, as that known as "Liquid Gold," which consists essentially of a solution of a sulpho-resinate of gold in suitable solvents, or of a mixture of the two materials.

Whilst either of the above two kinds of decalcomania may be employed for the application of vitrifiable enamel decorations, it has been found that the successful application of decorations in gold cannot be achieved with decalcomanias in which the design is applied over the support film, but that it is essential to employ decalcomanias of the covercoat type, that is to say those in which the support film overlies the design.

The covercoat support film at present used on decalcomanias carrying gold designs is of a cellulosic nature and based on ethyl cellulose. Such a covercoat enables a bright gold decoration to be obtained on a glass or pottery base after firing, but is unfortunately not sufficiently flexible for ease of handling and, consequently, difficulty is often experienced in applying a design film to an article of complicated shape such as is frequently produced in the pottery industry.

On the other hand, covercoat-type decalcomanias, carrying designs in ceramic color or vitrifiable enamel, usually employ resinous or resin-based covercoats, such, for example, as an acrylic resin, which possesses the physical characteristics, such as flexibility, required for ease of application to complicated shapes and is consequently much to be preferred to cellulose-based materials.

Whilst resin-based covercoat decalcomanias have proved eminently suitable for use for applying ceramic colors, attempts to use such covercoats with gold-design-carrying decalcomanias have met with little or no success, mainly owing to the fact that reaction occurs between the gold design film and the covercoat which destroys not only the brightness of the fired gold film, but also its adherence to the base. It appears, moreover, that the usual solvents employed in the covercoat solution tend to dissolve the gold film and separate the resinous material in the gold composition.

The principal object of this invention is to overcome the above disadvantage in the use of resin-based cover-

2

coats and to enable such covercoats to be successfully used with decalcomanias carrying a design in gold.

Another object is to provide an improved gold-carrying decalcomania for use in the decoration of heat-resisting bases.

A further object of the invention is to provide an improved method of decorating a heat-resisting base with designs in gold.

With these and other objects in view, the invention 10 provides a decalcomania or transfer of the covercoat support film type in which the design is applied to a paper backing beneath the support film which constitutes the covercoat, which comprises a design layer formed of, or comprising a gold-containing composition, a covercoat 15 support film formed of a resin-based material, and, between the design layer and the covercoat film, a protective layer of an oxidizable or polymerizable material which is impervious to the covercoat material and is inert to the gold in the design layer.

20 By this means the disadvantages hitherto associated with resin-based covercoats on gold-design-carrying decalcomanias are entirely obviated as the intermediate protective layer prevents penetration of any solvents from the covercoat film to the gold design and also prevents 25 any reaction between the resin in the covercoat and the gold in the design layer during firing of the design on the base.

The invention also comprises a method of making a 30 decalcomania or transfer of the covercoat support film type including the steps of applying a gold-containing design layer to a paper backing, applying, to the said layer, an intermediate protective layer of an oxidizable or polymerizable material which is inert to the gold in the design layer and then applying to said intermediate layer 35 a covercoat support film formed of a resin-based material, said intermediate layer also being impervious to said covercoat material.

The intermediate protective layer may consist of an 40 alkyd resin, a phenolic resin, or a urea resin.

45 The covercoat support film may consist of any known resin-based covercoat solution at present used with ceramic color or enamel decalcomanias, such, for example, as a methyl methacrylate resin-based film.

In carrying out the invention in practice, the intermediate polymerizable protective layer may advantageously have the following composition, namely,

|                                                   | Percent |
|---------------------------------------------------|---------|
| Short oil alkyl resin (60% non-volatile in xylol) | 25.00   |
| Cellulose nitrate                                 | 6.25    |
| Plasticizer                                       | 6.25    |
| High boiling solvent                              | 62.50   |

A suitable covercoat support film may have the following composition:

|                           | Percent |
|---------------------------|---------|
| Methyl methacrylate resin | 54.00   |
| Aromatic hydrocarbon      | 36.00   |
| Phthalate plasticizer     | 2.40    |
| Diluent                   | 7.60    |

60 The gold-containing design layer used may be any known and commercially available "Liquid Gold" preparation. The composition of such materials forms no part of this invention, and it will suffice to say that in general they are composed of a sulpho-resinate of gold in suitable solvents, usually with the addition of the resinates of other metals. The design layer may consist solely of a gold preparation, or of a mixture of such a preparation and one or more ceramic colors or vitrifiable enamels, according to the requirements of the final desired decoration.

70 The invention is illustrated, by way of example, in the

accompanying diagrammatic drawing, the single figure of which represents a section through a transfer or decalcomania embodying the invention.

In the drawing, 1 represents a gummed paper backing, the adhesive layer being represented at 1a; 2 a design film or layer formed of a "Liquid Gold" preparation, 3 an alkyd resin protective layer of the above specified composition, and 4 a covercoat support film also having the composition given above.

The layers 2, 3 and 4 are each preferably applied by the silk-screen printing method, the gold design layer being applied through a plain weave mesh screen having 200 strands to the inch. A coarser mesh screen having 90 strands to the inch is preferably used for applying the composition given above.

Whilst in the above one example of the invention has been described, it is to be understood that the invention is in no way limited to, or by, this example, but that modifications may be made thereto without departing from the scope of the invention. For example, any other suitable "Liquid Gold" design preparation may be used, and linseed oil or tung oil or another polymerizable resin other than an alkyd resin may be employed. Again, the covercoat may have a different composition from that given above. Furthermore, the constituent layers of the decalcomania need not be applied by the silk-screen printing method but any other suitable method, such as spraying or painting may be used instead.

It is, moreover, to be understood that the invention is intended to include within its scope a method of decorating a heat-resisting base with a design or decoration in gold with the use of decalcomania in accordance with,

or when made by the method of, the invention and any heat-resisting base when so decorated.

What we claim is:

1. A water release transfer of the covercoat support film kind comprising a paper backing carrying a layer of a water-soluble adhesive, a design layer comprising a sulfo-resinate of gold on the said layer of water-soluble adhesive, a protective layer comprising a material selected from the group consisting of alkyd resins, phenolic resins, and urea resins covering said design layer and a flexible covercoat film formed of resin-based material covering the said protective layer including the edges of said protective layer and the edges of said design layer, the protective layer being impervious to the covercoat film and inert to the gold in the design layer.

#### References Cited

##### UNITED STATES PATENTS

|           |         |                  |       |         |
|-----------|---------|------------------|-------|---------|
| 1,634,617 | 7/1927  | Hart             | ----- | 156—240 |
| 1,658,263 | 2/1928  | Stanley          | ----- | 40—21   |
| 1,888,154 | 11/1932 | Allen et al.     | ----- | 117—3.3 |
| 2,017,367 | 10/1935 | Kurz             | ----- | 117—3.3 |
| 2,124,232 | 7/1938  | Kittredge et al. | ----- | 117—122 |
| 2,970,076 | 1/1961  | Porth            | ----- | 156—89  |
| 3,156,580 | 11/1964 | Howard           | ----- | 117—75  |

##### FOREIGN PATENTS

784,966 10/1957 Great Britain.

30 EARL M. BERGERT, *Primary Examiner.*

H. F. EPSTEIN, *Assistant Examiner.*